

Nov. 5, 1929.

F. MARTINDELL

1,734,737

## METHOD OF AND APPARATUS FOR COATING STRAND MATERIAL

Filed Aug. 14, 1928

Fig. 1.



Fig. 2.



Fig. 3.



Inventor  
Frank Martindell  
by Hebertson Att'y.

## UNITED STATES PATENT OFFICE

FRANK MARTINDELL, OF RIVERSIDE, ILLINOIS, ASSIGNOR TO WESTERN ELECTRIC COMPANY, INCORPORATED, OF NEW YORK, N. Y., A CORPORATION OF NEW YORK

## METHOD OF AND APPARATUS FOR COATING STRAND MATERIAL

Application filed August 14, 1928. Serial No. 299,462.

This invention relates to a method of and apparatus for coating strand material, and more particularly to a method of and apparatus for coating wire.

5 In the past, wire has been coated with tin in many instances by passing the wire through a bath of the coating material and then drawing the coated wire through a die to remove the excess of the coating material.

10 Objects to this invention are to provide an economical and efficient method of and apparatus for coating strand material.

In accordance with the general features of the invention, one embodiment thereof consists of a member for whirling or revolving an advancing portion of a wire that has received a molten tin coating. The whirling of this tin coated portion centrifugally removes an amount of the tin, depending upon the 20 rate of the whirling and the speed of advancement. A guard is preferably placed over the whirling portion to confine the movement of the removed coating material.

It is believed that a clear understanding of 25 the invention may be had from the following detailed description taken in connection with the accompanying drawings, wherein

Fig. 1 is a longitudinal view of a tinning machine embodying features of the invention 30 for removing excess molten tin from a wire and which may be employed for practicing the improved method;

Fig. 2 is an enlarged, fragmentary vertical sectional view of the excess tin removing 35 apparatus shown in Fig. 1, and

Fig. 3 is a cross section of the same apparatus taken on line 3—3 of Fig. 2.

Referring now to the drawings in detail 40 wherein like reference numerals indicate similar parts, the numeral 10 indicates the framework of any ordinary and suitable tinning machine for tinning a wire 11 extending from a supply spool 12 to a suitably driven take up spool 13 by way of guide pulleys 16, 45 17, 18, and 19. A resiliently adjustable tension arm 14 and a brake 15 co-operating with the supply spool 12 maintain a suitable tension in the wire. A hook 20 directs the wire through a molten bath of tin 21 maintained 50 within a suitably heated container 22. From

the bath the wire passes through a device designated generally as 23 for producing a uniform tin coating, then through a water bath 24, and finally on to the take up spool 13.

The device 23 for producing the uniform 55 coating includes a guide 27 for receiving the wire immediately after it is drawn from the molten tin bath 21. From the guide 27, the tin coated wire 11 passes over an eccentric, rotatable member or finger 28 provided with 60 a groove 29 for receiving the wire, the member 28 being located at some distance from the guide 27. A cylindrical member 30 secures the member or finger 28 and rotates within a support 31 secured to a portion of 65 the frame 10 of the tinning machine. A pulley 32 secured to the cylindrical member 30 and driven by suitable means such as a belt (not shown) serves to rotate the cylindrical member and the finger 28. A guide 33 is provided within the cylinder 30 for receiving the wire 11 after passing over the eccentric finger 28, and from the guide 33 the wire passes to the water bath 24. A guard 34 suitably secured to the support 31 and the framework 10 70 of the machine is mounted over the portion of the wire 11 extending from the guide 27 to the guide 33. A door 35 provided with 75 hinges 36 permits access to the described parts.

The operation of the apparatus involves 80 the principle of centrifugally removing an amount of the molten tin coating by whirling or revolving the freshly tinned portion of the wire. The rotating finger 28 revolves the ever changing portion of the wire extending 85 between the guides 27 and 33 in the form of a loop, and obviously by regulating the speed at which the finger 28 is rotated the amount of tin thrown off the wire and thereby the thickness of the tin coating may be controlled. The groove 29 for receiving the wire in the rotating finger is slightly eccentric to the line of travel of the wire in order to effect the aforementioned revolving of the loop between the guides 27 and 33, and a constant tension is maintained in this loop by the adjustable tension arm 14 and brake 15 co-operating with the supply spool 12 or by other suitable means. Obviously by whir- 90 95 100

ing the freshly coated wire 11 as it passes between the guides 27 and 33, any excess tin is removed and a uniform coating of tin may be left on the wire. This method of centrifugally displacing the excess tin without the use of dies produces a resulting uniform coating in an obviously economical manner.

It is, of course, to be understood that the invention is not to be limited to the specific embodiment described for tin coating wire, but is susceptible to other applications included within the scope of the appended claims.

What is claimed is:

15 1. A method of coating strand material, consisting in advancing the material through a coating substance, and revolving the material after it has advanced through the substance to remove an amount of the coating 80 substance.

20 2. A method of coating strand material, consisting in longitudinally drawing the material through a bath of a coating substance, and revolving the material in a direction 85 transverse to the direction in which it is drawn and after the material has emerged from the coating bath to remove an amount of the coating substance.

25 3. A method of producing a uniform coating on strand material, consisting in immersing the material in a bath of a coating substance, and then revolving an everchanging portion of the material to remove excessive 90 coating substance and produce an evenly distributed covering.

30 4. In an apparatus for coating strand material, a container with a coating substance, means for drawing the material through the coating substance, and means for revolving the material after it has been drawn through 95 the coating substance to remove an excess thereof to produce a uniform covering.

40 5. In an apparatus for coating strand material, a container having a bath of a coating substance through which the material is drawn, guides for directing the material out of the bath and for determining the course 100 of the material, means for maintaining a tension in the material, and means for revolving the portion of the material between the guides to centrifugally remove excessive coating substance retained by the material.

45 6. In an apparatus for tinning wire, a container of molten tin through which the wire is drawn, guides for directing the wire out of the molten tin, and a rotating member for revolving the portion of the wire between the guides to centrifugally remove excessive molten tin retained by the wire.

50 7. In an apparatus for coating strand material, a container with a coating substance, means for drawing the material through the coating substance, a rotatable means through 105 which the material is drawn after it has passed through the coating substance to re-

75 80 85 90 95 100 105 110 115 120 125 130

volve the material to remove excess coating substance and a guard over the revolving material to confine the movement of the removed coating substance.

In witness whereof, I hereunto subscribe 70 my name this 26th day of July, A. D. 1928.

FRANK MARTINDELL.

75

80

85

90

95

100

105

110

115

120

125

130